

## UNITED STATES PATENT OFFICE.

CHARLES W. STUART, OF CHICAGO, ILLINOIS.

## CLEANING COMPOSITION.

No Drawing.

Application filed June 27, 1924. Serial No. 722,675.

This invention relates to cleaning compositions or compounds and more particularly to a cleaning composition or compound for removing oil, grease, dirt, and the like from metal surfaces to be painted, enameled or plated, although it is of general utility for any cleaning purpose.

The cleaner forming the subject matter of the invention has the desirable advantages of harmlessness and safety in use. It is preferably dissolved or mixed in water in tanks or vats suitable for dipping or otherwise immersing the metal articles to be cleaned. It has no deleterious effects upon the metal of tank or article, nor does it clog or deteriorate sewers or wastepipes into which the refuse from the cleaning vats may be poured.

Essentially the action of the cleaner is to cut the mineral oil from the metal to be cleaned or to combine with the oil in such manner that it will readily emulsify in water in which the metal may be immersed or rinsed.

It is therefore one object of the invention to provide a cleaning compound adapted to remove mineral oil and other oils, greases and the like from metal or wood without injury to the material or to the user, and to provide a cleanser that will emulsify in water together with the mineral oil or grease which it has removed or dissolved.

Another object is to provide a novel method of combining the ingredients whereby I attain the desirable results and functions.

A further object is to provide a unique method of removing mineral and other oils and grease from wood or metal or from other materials, for any purpose, for instance, such as that described.

Still further objects and advantages will appear from perusal of the detailed description of a certain form of my invention and from the claims.

In a simple form the cleaning composition or material may consist of a soluble oil base to which a suitable alkali is added. By the term, soluble oil base, is meant a treated oil which has the property of combining with mineral oil and causing it to emulsify with water. It may be unsaponified or either partially or wholly saponified animal or vegetable oil, or both, and to cause emulsification, various agents may be used, such solvents as alcohol, phenol, water and

mineral oil, being particularly valuable in this connection.

The approximate formulæ of a number of soluble oil bases are hereinafter given, the majority of which can be procured upon the open market. They do not, except in combination, form part of the invention hereof.

1.

|               | Per cent. |
|---------------|-----------|
| Rosin oil     | 26        |
| Oleic acid    | 40        |
| Alcohol       | 20        |
| Soda solution | 14        |

2.

|               | Per cent. |
|---------------|-----------|
| Lard oil      | 52        |
| Carbolic acid | 24        |
| 35° Caustic   | 24        |

3.

|            | Per cent. |
|------------|-----------|
| Rosin      | 7 lbs.    |
| Kerosene   | 2 gals.   |
| Caustic    | 2 lbs.    |
| Ammonia    | 2 gals.   |
| Oleic acid | 150 lbs.  |
| Alcohol    | 2 gals.   |

While the majority of soluble oil bases are not in themselves completely emulsifiable the use of any base which does completely emulsify in water without additional ingredients appears to greatly enhance the functioning of the cleaner.

The difference between a soluble oil and a soluble oil base is this: In the usual process of making soluble oil, one part of soluble oil base is mixed with from four to six parts of mineral oil and the resultant mixture becomes emulsifiable in water in its entirety and is called a soluble oil for this reason. If mineral oil is added to a soluble oil base to an amount to completely saturate the base, no greater amount of mineral oil will be taken up by the base and any excess of mineral oil beyond that necessary to completely saturate the base will not emulsify in water and will float on the top thereof. The function of my cleaner depends upon the affinity of the soluble oil base therein for more mineral oil other than that with which it may be mixed as a so-called "catalytic" agent and, therefore, when the cleaner comes in contact with mineral oil or grease on a part to be cleaned, it will absorb all mineral oil therefrom and become a soluble oil which will immediately flash into an emulsion in

water. Thus it will be apparent that the cleaning action of my cleaner depends upon the property of the soluble oil base in the cleaner to absorb or take up an additional 5 quantity of mineral oil from the article to be cleaned before it reaches its saturation point. In other words, if a soluble oil base which had the property of combining with eight times its weight of paraffin oil, were used 10 and mixed with six parts of paraffin oil prior to its use in a cleaner, the resultant oil would only have the property of taking up an additional two parts of paraffin oil from the article to be cleaned. It will be understood, of course, that the soluble oil base must of itself 15 be soluble or emulsifiable in water.

To the soluble oil base, an alkaline material of detergent qualities is added, which, for the work of removing oil and grease is 20 preferably a phosphate of soda, such as tri-sodium phosphate. Di-sodium phosphate is also valuable, and other like alkalies could be used. The soluble oil base and the alkalies are thoroughly mixed and worked together to form a homogeneous mixture in 25 suitable proportions which may vary over a wide range. For instance, the soluble oil base may be varied between 1% and 20% of the final product, and the alkali such as phosphate of soda, between 30% and 95% of the 30 final product. These compositions will have the property of dissolving or removing the grease or oil from the article and whereby it may emulsify and be carried in solution or 35 substantial solution in water.

After thoroughly mixing the phosphate of soda or other alkali with the soluble oil base, a dry, or substantially dry powder may be added to pick up or absorb any surplus oil or 40 moisture contained therein. The addition of this powder, drier, or absorbent is unnecessary to the functioning of the cleaner, but renders it easier to handle because the product formed of the soluble oil base and alkali 45 is generally of a mushy consistency which is usually undesirable in handling for packing or use. I have found it best to use materials which are not abrasive in their character, such as dextrine, or soda ash. Soda ash is to 50 be preferred because of its low cost and high solubility. This drying, filling, or absorbing ingredient may be added in quantities varying between five and sixty per cent of the final product as may be desired.

55 For ordinary metal cleaning, the most desirable ingredients and quantities I have found to be; soluble oil base 6%, phosphate of soda 82%, and soda ash 12%.

60 In using the cleaner it is preferably added to water and the mixture heated to the boil-

ing point although hot water may be used initially. Approximately four ounces of cleaner may be proportioned to each gallon of water, and after thorough mixing, the articles to be cleaned may be plunged into 65 the solution singly or in baskets as convenient, depending upon their size, etc. During this operation, the mixture is preferably maintained at the boiling point.

Just what chemical reactions or combinations take place between the various ingredients which form the soluble oil base, or between the base and phosphate or other alkali, and between the composition cleaning material and the oil and water, I can only 70 speculate and speculating would serve no useful purpose herein. Suffice it to say that by following this specification, those skilled in the art will be able to duplicate the material and results. There does seem, however, to be some chemical combination between the ingredients and there is, without doubt, a certain affinity of the mineral oils for the cleaner, while the addition of a small quantity of a mineral oil to the soluble oil base during its manufacture has an action apparently similar to that of a catalytic agent, facilitating solution or emulsification of the cleaner and oils or greases 80 in water. The effect of the cleaner on the mineral oil may be to dissolve it chemically or mechanically and when the resultant product passes into water it appears to emulsify although the mixture may be chemically rather than mechanically dissolved 85 therein.

I have described my invention in one illustrative form and not by way of limitation, since various changes may be made within its scope without departing from its spirit 100 or the purview of the appended claims.

I claim:

1. A cleaning composition containing a soluble oil base, and phosphate of soda.
2. A cleaning composition containing a soluble oil base, and tri-sodium phosphate.
3. A cleaning composition containing a soluble oil base, an alkali having detergent properties, and a filler.
4. A cleaning composition containing a soluble oil base from 1 to 20%, tri-sodium phosphate from 30-95%, and soda ash from 5-60%.
5. A cleaner containing 6% of soluble oil base, 82% of a phosphate of soda, and 12% of soda ash.

In testimony whereof I affix my signature at 10 S. La Salle St., Chicago, Ill.

CHARLES W. STUART.